

# UNITED STATES PATENT OFFICE.

WILLIAM A. FAIRBURN, OF SHORT HILLS, NEW JERSEY, ASSIGNOR TO THE DIAMOND MATCH COMPANY, OF CHICAGO, ILLINOIS, A CORPORATION OF ILLINOIS.

## MATCH-IGNITION MATERIAL.

1,206,827.

Specification of Letters Patent.

Patented Dec. 5, 1916.

No Drawing.

Application filed April 6, 1915. Serial No. 19,552.

*To all whom it may concern:*

Be it known that I, WILLIAM A. FAIRBURN, a citizen of the United States, and resident of Short Hills, in the county of 5 Essex and State of New Jersey, have invented certain new and useful Improvements in Match-Ignition Materials, of which the following is a specification.

This invention concerns a match-ignition 10 material designed more especially for use with or as an integral part of match receptacles and the like.

The material is in the form of a solid 15 block or body comprising a composition of matter, which, when molded into shape and allowed to harden, provides and insures an ignition surface for matches of different kinds,—to wit, those that may be struck on any ordinary rubbing surface and those that 20 may be struck on specially-prepared chemical surfaces—which said ignition surface is characterized by its smoothness, permanence and efficiency under widely varying conditions of temperature and relative hu- 25 midity.

Ignition material embodying my invention does not melt or run when it is subjected to great heat; and when such material is molded into or otherwise applied to 30 a suitable fire-proof holder, base or marginal frame member, which covers and protects the edges and corners of the block, the material cannot be ignited by flame. During extremely high humidity, with relatively high or low temperature or fluctuations of temperature which subject the material alternately to the dew point, the smoothness and ignition efficiency of the surface of the composition is unimpaired. 35 The block can be immersed in water and cleansed without injuring its smoothness or shape; the small amount of water the material may absorb when being washed drying out immediately after removing it from the 40 water. Such material remains permanently 45

hard, and it does not wear away appreciably, or lose its ignition efficiency, by the striking of thousands of matches thereon.

The ignition material possessing the characteristic properties and advantages above 50 mentioned consists essentially, of resin, dextrin, antimony sulfid, plaster of Paris and amorphous phosphorus (or other allotropic form of phosphorus or compound of phosphorus), in certain proportions, the whole 55 being intimately mixed together and sufficient water added thereto to make a stiff paste. The mixture is molded into any appropriate form and permitted to harden, the surface of the resulting block or body 60 being smooth, since there is no abrasive material used therein.

The ingredients entering into the composition are combined in about the proportions (by weight) stated, viz.:—

|                      |              |
|----------------------|--------------|
| Resin                | 4 parts.     |
| Dextrin              | 1 part.      |
| Plaster of Paris     | 16 parts.    |
| Antimony sulfid      | 12 parts.    |
| Amorphous phosphorus | 70 16 parts. |

These ingredients are thoroughly mixed and water is added thereto to make a stiff paste as above mentioned.

As above indicated instead of amorphous 75 phosphorus, any other allotropic form of phosphorus or compound of phosphorus may be used as an ingredient of the mixture, without departing from the invention defined in the appended claim.

I claim—

The herein described match ignition material composed of resin, dextrin, plaster of Paris, antimony sulfid and amorphous phosphorus, combined in about the proportions 85 specified.

Signed at New York in the State of New York this 5th day of April A. D. 1915.

WILLIAM A. FAIRBURN.